

H. E. HONEYWELL.  
PROCESS OF VARNISHING BALLOONS.  
APPLICATION FILED FEB. 21, 1918.

1,281,374.

Patented Oct. 15, 1918.



Attest.  
Charles A. Becker

Inventor:  
Harry E. Honeywell,  
by Ripley Kingsland  
his attorney.

# UNITED STATES PATENT OFFICE.

HARRY E. HONEYWELL, OF ST. LOUIS, MISSOURI.

## PROCESS OF VARNISHING BALLOONS.

1,281,374.

Specification of Letters Patent. Patented Oct. 15, 1918.

Application filed February 21, 1918. Serial No. 218,533.

To all whom it may concern:—

Be it known that I, HARRY E. HONEYWELL, a citizen of the United States, residing at the city of St. Louis and State of Missouri, have invented a new and useful Process of Varnishing Balloons, of which the following is a specification.

This invention relates to the process of varnishing balloons.

10 An object of the invention is to provide a novel method or mode of procedure for treating or varnishing the cloth or fabric used in the manufacture of balloons.

Another object of the invention is to provide 15 a novel composition for use in treating or varnishing the cloth or fabric.

By my new process the cloth is first sized with a varnish, the sizing being effected by submerging the cloth within a quantity of 20 varnish in a proper receptacle until the cloth has become saturated and impregnated with the varnish.

After having been submerged for a sufficient time to become thoroughly saturated 25 and impregnated with the varnish the sizing is completed by passing the cloth between rollers, similar to the rollers of a wringer, to press out and remove from the cloth all 30 excess quantity of varnish and leaving the cloth properly sized with the varnish in which it had been submerged.

After the cloth has been passed between the rollers it is fastened upon a rack including a number of rigid parallel rods, 35 lines, poles or other suitable supports to hold the cloth in such position that the threads are straight and to prevent sagging of the material or stretching of any portion of the material beyond other portions thereof. 40 The cloth is maintained on the rack until it has become sufficiently dried, and then may be cut and sewed together to form the balloon. It is preferable that the balloon be constructed on the French block 45 system so that the seams or lines of stitching are not continuous from the top to the bottom of the balloon. The method of the manufacture of the balloon on the French block system is much more convenient and 50 is preferable in other respects over the construction in which the seams or lines of stitching are continuous from top to bottom.

The drawing is a sectional view of a portion of the balloon illustrating the arrangement 55 of the substances or material applied to the balloon cloth.

The solution in which the cloth is immersed as described, consists of a mixture of linseed oil, litharge and yellow ocher, in approximately the proportions of one-half 60 pound of litharge and one-half pound of yellow ocher to each gallon of oil. The mixture of these ingredients is boiled until reduced to a proper consistency so that when the cloth is immersed therein the cloth will 65 become thoroughly saturated and impregnated.

The sizing applied to the cloth in the manner described closes the openings and interstices in the cloth so that when the 70 edges of the sections of cloth are sewed together the sizing is in and between the contacting portions of cloth which are sewed together as shown at 1 in the drawing.

After the cloth has been treated and dried, 75 cut and sewed to form the balloon, it is then treated with one or more applications of varnish of the same character applied by hand by means of a cloth-sponge, or the like, to form a coat 2 which completely 80 closes any remaining pores, openings or interstices in the cloth forming the balloon. This coat of varnish thus applied covers the entire balloon and extends into and across the lines along which the blocks of cloth 85 are sewed together, thus completely filling and closing any holes or openings that might be caused by the stitching or sewing together of the cloth. The number of applications thus made to the surface of the 90 balloon varies according to the necessities of the case, determined by the character and kind of gas to be used. After the last application of varnish has thus been made and while the surface of the balloon is yet in 95 a tacky state, it is treated by a silverizing process. The silverizing process consists in placing upon the balloon, before the last application of varnish has become thoroughly dried and while the varnish is yet 100 in a tacky condition, a coat 3 of silverizing substance in order to provide a perfectly smooth and finished surface and completely fill and close any remaining pores and perforations and render the balloon completely 105 gas-tight. The silverizing process which I prefer is a novel composition produced by the admixture of aluminum dust or powder and powdered French chalk, or their equivalents, in the proportions approximately of one pound of aluminum dust or powder to 110 each two pounds of powdered French chalk.

These substances are thoroughly mixed together and are applied to the tacky surface of the balloon in a powdered form, thereby producing a perfectly smooth and finished 5 surface rendering the balloon surface ornamental and easy to handle, and eliminating all condition of tackiness.

This treatment also darkens the fabric and prevents or eliminates excessive or rapid 10 contraction and expansion of the gases in the balloon when passing from a cloud into the clear sky and the full heat of the sun intermittently.

In practice, I prefer to complete the upper 15 and lower halves of the balloon envelop separately, each being constructed on the French block system and each half of the envelop being finished with the final silverizing coating before the two halves of the balloon are 20 sewed together to complete the balloon. This system of manufacture is much more convenient and the two halves of the balloon may be handled independently more readily and with less trouble than is possible when 25 the entire envelop is completed before the final silverizing coating is applied.

It will be understood that the order of 30 procedure may be varied in unessential particulars and that equivalent ingredients may be used in the place of the ones mentioned without departure from the principles of 35 the invention. I do not restrict myself to precise proportions or ingredients or to other unessential limitations, but contemplate such variations as are within the principles of the invention as set forth in the appended claims.

What I claim and desire to secure by Letters Patent is:—

40 1. The process of making balloons, which consists in submerging the cloth in a sizing varnish, removing the excess varnish from the cloth, drying the cloth; preventing stretching of any portion beyond other portions thereof while the cloth is being dried; 45 sewing the cloth to form the balloon; applying a coating of varnish to the surface of the balloon; and then when the cloth is yet in a tacky condition applying thereto a powdered silverizing coating which forms a smooth or sleek surface.

2. The process of making balloons, consisting in sizing the balloon cloth with a mixture composed of linseed oil, litharge and 55 ocher; drying the cloth; sewing the cloth to form the balloon; applying a coating of varnish to the surface of the balloon; and then applying to the surface of the balloon while in a tacky condition a powdered mixture consisting of aluminum dust and powdered French chalk.

3. The process of making balloons, consisting in sizing the balloon cloth in a boiled mixture composed of linseed oil, litharge 60 and ocher in the approximate proportions

of one-half pound litharge and one-half pound ocher to each gallon of oil; drying the cloth; sewing the cloth to form the balloon; applying a coating of varnish to the surface of the balloon; and then applying 70 to the surface of the balloon while the surface is in a tacky condition a powdered mixture including aluminum dust and powdered French chalk which mixture forms a smooth surface upon the balloon.

4. The process of making balloons, consisting in sizing the balloon cloth with a substance to close the pores and interstices in the cloth; drying the cloth; sewing the cloth to form the balloon; producing a tacky 80 surface on the balloon by a coat of varnish; and applying to the tacky surface of the balloon a mixture which adheres to the tacky surface and forms a smooth surface.

5. In the manufacture of balloons, the 85 process of making the balloon which consists in sizing the balloon cloth in a boiled mixture comprising linseed oil, litharge and ocher in the approximate proportions of one-half pound litharge and one-half pound 90 ocher to each gallon of oil; passing the cloth between rollers to remove the excess of the mixture from the cloth and leave the cloth sized with the mixture; drying the cloth; sewing the sized cloth to form the balloon, 95 and applying a coat of varnish to the surface of the balloon.

6. In the manufacture of balloons, the process of making the balloon which consists in sizing the balloon cloth in a boiled 100 mixture comprising linseed oil, litharge and ocher in the approximate proportions of one-half pound litharge and one-half pound ocher in each gallon of oil; passing the cloth between rollers to remove the excess of the 105 mixture from the cloth and leave the cloth sized with the mixture; drying the cloth; sewing the sized cloth to form the balloon; producing a tacky surface on the balloon by applying a coat of varnish; and applying 110 to the tacky surface of the cloth a silverizing mixture which adheres to the sized cloth and forms a smooth surface.

7. In the manufacture of balloons, the 115 process of making the balloon which consists in sizing the balloon cloth in a boiled mixture comprising linseed oil, litharge and ocher in the approximate proportions of one-half pound litharge and one-half pound ocher to each gallon of oil; passing the cloth between rollers to remove the excess of the mixture from the cloth and leave the cloth sized with the mixture; drying the cloth; sewing the cloth to form the balloon; producing a tacky surface on the balloon by applying a coat of varnish; and applying to 120 the tacky surface of the cloth a silverizing mixture including aluminum dust and powdered French chalk.

8. In the manufacture of balloons, the 130

process of making the balloon which consists in sizing the balloon cloth in a boiled mixture comprising linseed oil, litharge and ocher in the approximate proportions of 5 one-half pound litharge and one-half pound ocher to each gallon of oil; passing the cloth between rollers to remove the excess of the mixture from the cloth and leave the cloth sized with the mixture; drying the cloth;

sewing the cloth to form the balloon; producing a tacky surface on the balloon by a coat of varnish; and applying to the tacky surface of the cloth aluminum dust and powdered French chalk in the proportions of one pound of aluminum dust to each two 15 pounds of powdered French chalk.

HARRY E. HONEYWELL.